

## UNITED STATES PATENT OFFICE

LOUIS J. CONRAD, OF BROOKVILLE, INDIANA

## PROCESS OF TREATING LUMBER

No Drawing.

Application filed December 11, 1928. Serial No. 325,393.

This invention relates to a process for treating lumber and more particularly to a process for steaming black walnut boards.

Black walnut boards, as they come from the sawmill in the woods are known as run of the mill boards and are usually of a uniform thickness and of varying widths. These run of the mill boards comprise a central longitudinal section, called the heart portion, and a longitudinal section at each side edge bounding the heart portion which is known as the sap portion. The sap portion appears to be lighter in color and of a slightly different texture from the heart portion. I have been unable to determine whether the difference in color and lack of homogeneity is due to retarded or undeveloped pigmentation in the sap portion, or whether the same is the result of the presence of rosin and other elements which do not occur or are present in smaller quantities in the heart portion.

It has been the practice to further treat these run of the mill boards at the factories by separating the sap portion from the heart portion and only using the heart portion, thereby necessitating the loss of the sap portion, or in only utilizing it in inferior grades of furniture and building trim. The foregoing practice is not only extravagant but it precludes the use of the entire width of the run of the mill boards.

The primary object of this invention is to provide, in a manner as hereinafter set forth, for simultaneously abstracting or devitalizing the harmful elements in the sap portion and uniformly coloring run of the mill black walnut boards.

Another object of the invention is to provide, in a manner as hereinafter set forth, for producing a black walnut board which will not warp, crack or absorb moisture in the finished state; and which is capable of being polished or finished so as to present a uniform color and texture throughout when used in the manufacture of furniture or building trim.

Further objects of the invention are to provide, in a manner as hereinafter set forth, a process which is economically carried on

without danger of injuring the lumber; which does not require the use of expensive equipment or skilled labor and moreover does not utilize any chemicals or dyes in its operation.

In carrying out the invention, a suitable vat or treating receptacle of any desired material such as wood, cement or metal is utilized. The shape of the vat is preferably square and is provided with a suitable drain to withdraw the products of condensation accumulating therein. In the bottom of the vat is located a series of perforated pipes or individual jets as desired and said pipes or jets are connected to the steam supply pipes.

It has been found that wet, heavy or exhaust steam is preferable for the purpose of this invention, but the process will operate successfully with any kind of steam. It is not necessary nor advisable that the vat be pressure tight and it may be open at the top or may be provided with loose fitting cover. There will be no abnormal pressures developed in the vat and it is within the contemplation of the invention to treat the lumber at atmospheric pressure. A suitable support is secured to the bottom of the tank so as to provide a resting place for the lumber which is spaced from the steam jets in the bottom of the vat. The space will be filled with steam during the treatment of the lumber.

The run of the mill boards are piled in layers, one on top of the other and all of the boards will extend in the same direction. The boards are so arranged that the sap portion of each board in each layer will abut against and be adjacent to the heart portion of the boards in the overlying and the underlying layer. The varying widths of the run of the mill boards will accommodate the arrangement and moreover, will provide for spaces between the edges of each of the boards in the same layer, so as to compensate for the lateral expansion without altering the relative position with respect to the overlying and underlying layers. When the vat has been filled with the boards the entire mass is covered with black walnut saw dust and the steam is then allowed to enter the vat.

55

60

65

70

75

80

85

90

95

100

The steam slowly penetrates the mass of lumber and there will be a marked condensation within and on the surface of the pile of lumber. At the same time the condensed steam will react with the walnut saw dust and the products of the reaction will slowly percolate through the pile of lumber. In a vat 16' x 16' x 8' deep, satisfactory results have been obtained by steaming the charge for 36 hours. The time factor is variable according to the thickness of the boards, the size of the container, the quality of the steam and the seasoning given to the lumber prior to the treatment; and the aforementioned time is only given for the purpose of illustration without limiting the invention thereto.

When the boards have been treated the predetermined time the steam is turned off, the saw dust is removed and the boards are taken from the vat. It will be seen that there is a deposit on the surface of the boards where they have been in contact with each other. The corrosion is apparently due to the exudations from the sap portion of the boards. It will be further noted that the heart portion of the board appears to be lighter in color after the steaming, while the sap portion has taken on the same color and appears to be of the same texture as the heart portion. The boards are then dried, either by the natural process or by means of the conventional dry kiln. After the drying operation the boards are run through the planer, which removes the corroded surface and then they are made up into furniture or building trim. Upon the application of the usual finishes and polishes well known to the industry, the entire width of the board will be of a uniform color and will present a homogeneous texture.

It will be apparent from the foregoing description of the process that there are five factors functioning simultaneously during the treatment of the lumber, namely:—Heat in the presence of a vapor laden atmosphere; the percolation through the mass of lumber of the products of the reaction between black walnut saw dust and the steam vapor; the surface contact between heart and sap portion of the boards; the lateral diffusion of coloring matter from heart to sap portion in the same board; and the abstraction of elements which in the natural state impart heterogeneity to the boards. There is a sixth factor that may have an influence upon the success of the invention and that is the development of the latent pigmentation residing in the sap portion when subjected to the conditions of this process. It is within the contemplation of this process to claim only the cumulative effect of the six aforementioned factors in producing a black walnut board from run of the mill lumber which presents a uniform color and homogeneous texture.

What I claim is:—

A process of treating black walnut lumber which consists in piling run of the mill boards in layers extending in the same direction in a vat, with the boards of each layer arranged so that the sap portions thereof will be adjacent to and abut against the heart portion of the boards in the overlying and underlying layers, covering the resultant pile of boards with black walnut saw dust, and then steaming the pile.

In testimony whereof, I affix my signature hereto.

LOUIS J. CONRAD.

80

85

90

95

100

105

110

115

120

125

130